

1

2,846,307

## ISOXAZOLONE COUPLERS IN COLOR PHOTOGRAPHY

John Mathers Woolley, Manchester, England, assignor to Imperial Chemical Industries Limited, London, England, a corporation of Great Britain

No Drawing. Application October 17, 1955  
Serial No. 541,097

Claims priority, application Great Britain October 22, 1954

14 Claims. (Cl. 96—55)

This invention relates to colour photographic images and more particularly to a novel process for the production of colour photographic images by colour development in the presence of a colour coupler, to photographic developers and to photographic material containing such a coupler, and to photographic materials containing coloured images of the kind obtainable from such a colour coupler.

It is known that when a reducible silver salt image is developed with a primary aromatic amino developing agent in the presence of certain isoxazolones containing a reactive methylene group, dyestuffs of the azamethine class are obtained. Dyestuffs of this class in general have poor chemical stability and poor fastness to light.

We have now found that by developing the reducible silver salt with a colour developer in the presence of certain derivatives of isoxazolone which contain no reactive methylene group in the isoxazolone ring and which have not hitherto been known for use as colour couplers, a completely different process of colour coupling occurs.

According to our invention we provide a process for the production of colour photographic images which comprises developing an exposed gelatino-silver halide emulsion layer with a colour photographic developer in the presence of a colour coupler of the formula:



wherein Z represents the atoms required to complete a homocyclic, heterocyclic or polycyclic nucleus and R represents hydrogen or an acyl group.

The nucleus represented by Z may carry substituents for example halogeno, sulphonic acid, carboxylic acid, carboxylic ester or amide substituents. Z may represent for example the atoms required to complete a benzene nucleus, unsubstituted or substituted, that is to say the compounds may be  $\beta$ - $\gamma$ -benzisoxazolones which may carry substituents on the 1-, 4-, 5-, 6- or 7-positions. (The system of numbering used in this specification for  $\beta$ - $\gamma$ -benzisoxazolones is that given in the "The Ring Index" by Patterson and Capell published by Reinhold Publishing Corporation (1940) (No. 729).) As an example of a heterocyclic (and polycyclic) nucleus there may be mentioned the quinoline nucleus.

The colour coupler used in the process of our invention may be used in the developing solution or it may be included in a light-sensitive layer of a multilayer photographic material or in a non-light sensitive layer ad-

2

jacent to a sensitive layer or separated therefrom by a water-permeable colloid layer.

For the latter purpose an insoluble colour coupler may be used, or a soluble colour coupler enclosed in particles of water-insoluble, water-permeable material but it is preferred to use colour couplers which contain a substituent rendering them fast to diffusion, for example an alkyl chain of at least 5 carbon atoms and, if desired, a solubilising group.

10 The colour couplers used in the process of our invention may be made by the general processes known for use in the synthesis of  $\beta$ - $\gamma$ -benzisoxazolones for example by reducing the appropriate o-nitrocarboxylic acid or an ester thereof (for example o-nitrobenzoic acid, 3-nitrophthalic acid, 3-nitro-6-chlorophthalic acid, 2-nitro-4-sulphobenzoic acid, 5-octadecyloxy-6-nitro-trimellitic acid, 3-nitro-4-hydroxy-quinoline-2-carboxylic acid, ethyl ester or 2-nitroterephthalic acid) to the corresponding hydroxylamino compound, ring closing, and if desired, subsequently replacing the hydrogen atom attached to the nitrogen atom, by an acyl radical, for example by heating the compound with acetic anhydride, ethyl chloroformate, p-toluenesulphonyl chloride or phenylisocyanate.

15 Also, if desired, substituents may be introduced into the nucleus represented by Z, or substituents in the said nucleus may be modified by known reactions. For example when 3-nitrophthalic acid is used as starting material the 4-carboxy- $\beta$ - $\gamma$ -benzisoxazolone formed may itself be used as a colour coupler, or it may be converted to the corresponding 1-acetyl-, 1-phenylcarbamyl, 1-carbethoxy or 1-p-toluenesulphonyl-derivative by substitution on the nitrogen atom, or the carboxyl group in 4-carboxy- $\beta$ - $\gamma$ -benzisoxazolone or its 1-substituted derivatives may be modified for example by converting to the corresponding carboxylic acid chloride and reacting this with an alcohol such as octadecanol, or an amine such as octadecylamine or 1-amino-2-(N-methyl-N-octadecylamino)-benzene-5-sulphonic acid.

20 The colour photographic developers which may be used in the present invention include the mono-, di- and tri-amino-aryl compounds. Among the monoamino developers there may be mentioned amino-phenols and amino-cresols and their halogen derivatives and amino-naphthols.

25 30 35 40 45 The developers preferably used and giving the best results in connection with the present invention are the aromatic ortho- and para-diamines such as para-phenylene diamine and its substitution products.

The colour coupling which occurs in the process of our 50 invention when an exposed gelatino-silver halide emulsion is treated with a primary aromatic amino developing agent in the presence of one of the colour couplers as hereinbefore defined, proceeds by a surprising and wholly unexpected reaction in which the isoxazolone ring is split and an azo dyestuff is formed in which the residue of the oxidation product of the developing agent is attached to the nitrogen atom which previously formed the 1-nitrogen atom of the isoxazolone ring. For example when 1-phenylcarbamyl-4-carboxy- $\beta$ - $\gamma$ -benzisoxazolone is used as 55 60 the colour coupler, and p-diethylamino-aniline is used as developing agent, a dyestuff is formed which has the following formula:

65



It will be noted that the acyl substituent on the nitrogen atom in 1-position of the indazolone ring is split off during colour development.

According to a further feature of our invention therefore we provide a colour photographic element which contains in at least one emulsion layer, a colour image comprising a dyestuff of the formula:



wherein Z has the significance indicated above and X represents the group of atoms which together with the group  $\text{--NH}_2$  forms a primary aromatic amine which is capable of developing exposed silver halide emulsions.

By selection of suitable colour couplers, especially with regard to the atoms represented by Z in the above formula of the colour couplers, and by selection of suitable developing agents, it will be apparent that dyestuff images can be obtained with a wide range of hue, and it will also be apparent that by suitably after-treating the residual colour coupler, left after colour development a colour correcting masking image can be formed, or by selecting colour couplers which are themselves coloured, the residual colour coupler left after colour development can itself be utilized as a colour correcting masking image.

The dyestuff images formed by the process of our invention are superior to the known azamethine images in their chemical stability and their fastness to light and the process of our invention provides a simple method of obtaining colour photographic images of good fastness properties by direct development of an exposed gelatinousilver halide emulsion with a colour photographic developer.

The invention is illustrated but not limited by the following examples in which the parts are by weight:

#### Example 1

A developer solution is made up according to the following formula:

|                                          | Parts |
|------------------------------------------|-------|
| Sodium carbonate, anhydrous              | 16.2  |
| N:N-diethyl-p-phenylene-diamine sulphate | 0.75  |
| Potassium bromide                        | 0.25  |
| Sodium sulphite anhydrous                | 0.25  |
| $\beta:\gamma$ -Benzisoxazolone          | 0.5   |
| Water                                    | 250   |

A photographic silver halide emulsion layer which has been exposed to light is developed in this solution at 20° C. In the exposed parts of the layer, the silver halide is converted to metallic silver and the yellow azo dyestuff 2-carboxy-4'-diethylaminoazobenzene (sodium salt) is produced. This yellow azo dyestuff has much better stability to light than the azamethine dyestuffs produced by previously known colour development processes.

In place of the 0.5 part of  $\beta:\gamma$ -benzisoxazolone used in the developer solution in the above example there may be used the same weight of the N-acetyl derivative of this compound when the same dyestuff is produced, the acetyl groups being split off in the colour forming reaction.

In place of the N:N-diethyl-p-phenylene-diamine sulphate used in the developer solution in the above example there may be used 4-amino-3-methyl-N:N-diethylaniline, 4-amino-3-ethoxy-N:N-diethylaniline or p-phenylene diamine.

#### Example 2

In place of the 0.5 part of  $\beta:\gamma$ -benzisoxazolone used in Example 1 there is used 0.5 part of 4-carboxy- $\beta:\gamma$ -benzisoxazolone which may be prepared as follows:

31 parts of 3-nitro-phthalic acid are dissolved in 130 parts of water. The solution is added quickly to a solution of 100 parts of stannous chloride in 100 parts of 35% aqueous hydrochloric acid. Heat is evolved and a crystalline solid is formed. The mixture is cooled to 20°

C. and the crystalline product is filtered off, washed first with 20% aqueous hydrochloric acid and then with water and dried. 4-carboxy- $\beta:\gamma$ -benzisoxazolone is obtained in the form of pale yellow needle-shaped crystals (melting point 190–192° C.). The yellow azo dyestuff formed in the exposed parts of the silver halide emulsion layer is the sodium salt of 2:3-dicarboxy-4'-diethylamino-azobenzene.

The same dyestuff is obtained when in place of the 0.5 part of 4-carboxy- $\beta:\gamma$ -benzisoxazolone there is used 0.5 part of 1-acetyl-4-carboxy- $\beta:\gamma$ -benzisoxazolone (melting point 212° C.) which may be made by heating 4-carboxy- $\beta:\gamma$ -benzisoxazolone with acetic anhydride.

#### Example 3

In place of the 0.5 part of  $\beta:\gamma$ -benzisoxazolone used in Example 1, there is used 0.5 part of 6-carboxy- $\beta:\gamma$ -benzisoxazolone which may be prepared as follows:

16 parts of 2-nitro-terephthalic acid is stirred with 100 parts of water at 10° C. and 12 parts of zinc dust are added at such a rate that the temperature of the mixture does not rise above 15° C. When all the zinc dust has been added the mixture is stirred for a further 30 minutes at 15° C. and the mixture is then filtered. The residue is washed with 50 parts of water and sulphuric acid is added to the combined filtrates and washings until the mixture contains 10% free sulphuric acid. The solution so obtained is boiled and then cooled. 6-carboxy- $\beta:\gamma$ -benzisoxazolone which crystallises out is filtered off, washed with water and dried. The product is purified by stirring it with 20 parts of cold methanol for 15 minutes filtering off and recrystallising from methanol. The 6-carboxy- $\beta:\gamma$ -benzisoxazolone so formed does not melt below 300° C. The yellow azo dyestuff produced in the exposed parts of the photographic silver halide emulsion layer is 2:5-dicarboxy-4'-diethylamino-azobenzene. The same dyestuff is obtained when in place of the 0.5 part of 6-carboxy- $\beta:\gamma$ -benzisoxazolone there is used 0.5 part of 1-acetyl-6-carboxy- $\beta:\gamma$ -benzisoxazolone (melting point 190° C.) which may be made by heating 6-carboxy- $\beta:\gamma$ -benzisoxazolone with acetic anhydride.

#### Example 4

In place of the 0.5 part of  $\beta:\gamma$ -benzisoxazolone used in Example 1 there is used 0.5 part of 1-phenylcarbamyl-4-carboxy- $\beta:\gamma$ -benzisoxazolone which may be made as follows:

1 part of 4-carboxy- $\beta:\gamma$ -benzisoxazolone, 10 parts of dry dioxane and 1 part of phenylisocyanate are boiled together under a reflux condenser for 30 minutes. The mixture is cooled and the crystalline solid which separates from solution is filtered off, washed with methanol and ether and dried. The product melts at 190° C.

55

#### Example 5

In place of the 0.5 part of  $\beta:\gamma$ -benzisoxazolone used in Example 1 there is used 0.5 part of 1-carbethoxy-4-carboxy- $\beta:\gamma$ -benzisoxazolone which may be prepared as follows:

1 part of 4-carboxy- $\beta:\gamma$ -benzisoxazolone, 10 parts of chlorobenzene and 1 part of ethyl chloroformate are boiled together under a reflux condenser for 3 hours. The mixture is cooled and the crystals which separate from solution are filtered off, washed with benzene and dried. The product melts at 156° C.

#### Example 6

In place of the 0.5 part of  $\beta:\gamma$ -benzisoxazolone used in Example 1, there is used 0.5 part of 1-p-toluene-sulphonyl-4-carboxy- $\beta:\gamma$ -benzisoxazolone which may be prepared as follows:

1 part of 4-carboxy- $\beta:\gamma$ -benzisoxazolone is dissolved in 10 parts of pyridine and 2 parts of p-toluene-sulphonyl chloride are added. The mixture is heated to its boiling point and 10 parts of water are added. The mixture is

allowed to stand for 10 minutes and it is then poured into a mixture of 100 parts of water and 20 parts of hydrochloric acid. The syrup which is precipitated is separated and heated with 10 parts of methanol. The clear solution so formed is cooled when 1-p-toluenesulphonyl-4-carboxy- $\beta$ : $\gamma$ -benzisoxazolone crystallises out. The product is filtered off and dried. It melts at 206° C.

*Example 7*

1 part of the octadecyl ester of 1-acetyl-4-carboxy- $\beta$ : $\gamma$ -benzisoxazolone is dissolved in 5 parts of dibutyl phthalate and 1 part of the ammonium salt of sulphonated oleic acid is added. The solution so formed is added to 100 parts of a molten gelatino-silver halide emulsion at 40° C. The mixture is passed through a homogeniser. A layer of the mixture is then coated onto a film base and the layer is dried. The layer is exposed to light behind a step-wedge and then developed in a photographic colour developing solution containing N:N-diethyl-p-phenylene diamine as developing agent. The developed silver is bleached and the silver salts removed by a fixing bath. A yellow azo dyestuff image corresponding in gradation of density to the intensity of the incident light is obtained. The octadecyl ester of 1-acetyl-4-carboxy- $\beta$ : $\gamma$ -benzisoxazolone may be prepared as follows:

2 parts of 1-acetyl-4-carboxy- $\beta$ : $\gamma$ -benzisoxazolone and 10 parts of thionyl chloride are boiled under a reflux condenser for 2 hours. The excess thionyl chloride is distilled off and the carboxylic acid chloride dried in vacuo. A mixture of 1 part of the carboxylic acid chloride so formed, 2 parts of octadecanol and 10 parts of benzene are boiled under a reflux condenser for 2 hours. The mixture is cooled and the octadecyl ester of 4-carboxy- $\beta$ : $\gamma$ -benzisoxazolone which separates from solution, is filtered off, washed with benzene and dried. It melts at 71-72° C.

*Example 8*

In place of the 1 part of the octadecyl ester used in Example 7 there may be used 1 part of 1-acetyl- $\beta$ : $\gamma$ -benzisoxazolone-4-carboxyoctadecylamide which may be prepared as follows:

1 part of 1-acetyl- $\beta$ : $\gamma$ -benzisoxazolone-4-carboxylic acid chloride is dissolved in 10 parts of benzene and the solution is added to a solution of 3.5 parts of octadecylamine in 10 parts of pyridine and 10 parts of benzene. The solution is boiled for 5 minutes and the benzene and excess pyridine are then removed by vacuum distillation. The residue is dissolved in 10 parts of methanol and the solution is poured into a mixture of 100 parts of water and 10 parts of hydrochloric acid. The white precipitate so formed is filtered off, washed with water, then with methanol, and finally with ether and then dried. The product is recrystallised from methanol and then melts at 98-100° C.

*Example 9*

1 part of  $\beta$ : $\gamma$ -benzisoxazolone-4-carboxy-(2'-N-methyl-N-octadecylamino-5'-sulpho-benz)-amide is added to 5 parts of methanol and 4 parts of water and 0.4% aqueous caustic soda solution is added drop-wise until a clear yellow solution is obtained. The pH of this solution is adjusted to 8.0 by the addition of acetic acid or 0.4% aqueous caustic soda solution, and the solution is then added to 100 parts of a molten gelatino-silver halide emulsion. The emulsion is coated as a layer on a substrate and the layer is dried. The layer is exposed to light, developed with a solution of N:N-diethyl-p-phenylenediamine, the developed silver is bleached and the silver salts fixed. The layer is washed with water. An orange coloured azo dyestuff image is obtained.

The  $\beta$ : $\gamma$ -benzisoxazolone-4-carboxy-(2'-N-methyl-N-octadecylamino-5'-sulpho-benz)-amide used in this example may be prepared as follows:

2.2 parts of 1-acetyl- $\beta$ : $\gamma$ -benzisoxazolone-4-carboxylic acid chloride are dissolved in 18 parts of benzene and

the solution is added to a hot solution of 4.5 parts of 1-amino-2(N-methyl-N-octadecyl-amino)-benzene-5-sulphonic acid in a mixture of 10 parts of benzene and 8 parts of pyridine. The solvent is removed by vacuum distillation and the residue is dissolved in 20 parts of methanol. The solution is added to a mixture of 50 parts of ice and 20 parts of 35% hydrochloric acid. The gummy precipitate so formed is allowed to settle, and the supernatant liquid is decanted. The gummy residue is washed with water and then boiled with 100 parts of methanol. The solution so formed is cooled and the pale grey solid which is precipitated is filtered off and recrystallised from glacial acetic acid. The product melts at 212° C.

15

*Example 10*

In place of the 0.5 part of  $\beta$ : $\gamma$ -benzisoxazolone used in Example 1 there is used 0.5 part of 4-carboxy-5-chloro- $\beta$ : $\gamma$ -benzisoxazolone which may be prepared as follows: 20 36 parts of 3-nitro-6-chlorophthalic acid are dissolved in 130 parts of water. The solution is added quickly to a solution of 100 parts of stannous chloride in 100 parts of 35% aqueous hydrochloric acid. Heat is evolved and a crystalline solid is formed. The mixture 25 is cooled to 20° C. and the crystalline product is filtered off, washed first with 20% aqueous hydrochloric acid and then with water and dried. 4-carboxy-5-chloro- $\beta$ : $\gamma$ -benzisoxazolone is obtained in the form of pale yellow needle-shaped crystals (melting point 178° C.). The 30 yellow dyestuff formed in the exposed parts of the silver halide emulsion layer is the sodium salt of 2:3-dicarboxy-4-chloro-4'-diethylamino-azobenzene.

35

*Example 11*

In place of the  $\beta$ : $\gamma$ -benzisoxazolone used in the developing solution of Example 1 there are used 5 parts of a 10% aqueous solution of  $\beta$ : $\gamma$ -benzisoxazolone-6-sulphonic acid, when an azo dyestuff is formed which is bright yellow in colour in alkaline solution and bright reddish-magenta in acid solution.

The 10% aqueous solution of  $\beta$ : $\gamma$ -benzisoxazolone-6-sulphonic acid used in the above example may be prepared as follows:

45 2-nitrotoluene-4-sulphonic acid is oxidised in the usual manner with alkaline permanganate solution to give 2-nitro-4-sulphobenzoic acid.

2 parts of 2-nitro-4-sulphobenzoic acid are stirred in 200 parts of water containing 16 parts of ammonium 50 chloride, and 32 parts of zinc dust are added gradually to the cooled mixture at such a rate that the temperature of the mixture does not rise above 30° C. The mixture is stirred for 30 minutes at room temperature and then filtered. The filtrate is strongly acidified with hydrochloric acid and then boiled to ring-close the 2-hydroxyl-amino-4-sulphobenzoic acid to form the benzisoxazolone-6-sulphonic acid. The solution so obtained is just neutralised with sodium carbonate and filtered. The benzisoxazolone-6-sulphonic acid content of the filtrate is estimated by titration with N/2 sodium nitrite solution and water is then added to the filtrate to adjust the concentration of  $\beta$ : $\gamma$ -benzisoxazolone-6-sulphonic acid to 10% by weight.

65

*Example 12*

In place of the  $\beta$ : $\gamma$ -benzisoxazolone used in the developing solution of Example 1, there is used 0.5 part of hydroxy-quinoline-isoaxazolone prepared as described below. A photographic silver halide emulsion layer 70 which has been exposed to light is developed in the solution at 20° C. and the silver and silver halide in the exposed parts of the layer are removed. The yellowish-brown azo dyestuff in the exposed parts of the layer is changed to a bright magenta colour on treatment with 75 hydrochloric acid.

The hydro-quinoline-isoxazolone used in this example may be prepared as follows:

20 parts of 4-hydroxy-quinoline-2-carboxylic acid ethyl ester are dissolved in 18 parts of concentrated sulphuric acid below 30° C. 180 parts of a mixture of nitric acid and concentrated sulphuric acid (containing 10% of nitric acid) are gradually added to the solution and the mixture is stirred for 1 hour at 30° C. after the addition is complete. The solution is poured into 300 parts of ice and the yellow solid is filtered off and washed acid free. The filter cake is stirred into 60 parts of methanol, and the mixture is heated to the boil and filtered. The filter cake is washed with 60 parts of hot methanol and then recrystallised from 100 parts of acetic acid. 3-nitro-4-hydroxy-quinoline-2-carboxylic ethyl ester is thus obtained in the form of small yellow crystals which melt at 286° C. 4 parts of this product are stirred in 60 parts of water containing 2 parts of ammonium chloride, and 4 parts of zinc dust are gradually added during 15 minutes, the temperature of the mixture being kept below 30° C. by the addition of ice as required. The mixture is stirred for a further 15 minutes and then filtered. Sufficient hydrochloric acid is added to the filtrate until the mixture gives a strong blue colouration on Congo red paper. The turbid suspension so formed is boiled for 1 minute and then cooled and filtered and the mixture is stirred with 50 parts of normal sodium hydroxide solution. 1 part of decolourising charcoal is added and the suspension is filtered. The filtrate, is acidified and the precipitate is filtered off and dried. The product has the following formula:



Example 13

In place of the 1 part of  $\beta:\gamma$ -benzisoxazolone-4-carboxy - (2' - N - methyl - N - octadecylamino - 5' - sulphonylbenz) - amide used in Example 9, 1 part of 4:6-dicarboxy-7-octadecyloxy benzisoxazolone prepared as described below, is used. A yellow azo dyestuff image is obtained.

The 4:6-dicarboxy-7-octadecyloxybenzisoxazolone used in this example may be prepared as follows:

5-hydroxytrimellitic acid is converted to the trimethyl ester by heating it under a reflux condenser for 6 hours with methanol containing 5% by weight of anhydrous hydrochloric acid.

15 parts of the trimethyl ester are dissolved in 100 parts of oleum (containing 20% of free sulphur trioxide) at a temperature not higher than 30° C. The solution is stirred and cooled below 20° C. and 7.5 parts of potassium nitrate are added in portions at such a rate that the temperature does not rise above 20° C. When the addition of the nitrate is complete the solution is stirred for 30 minutes at 25° C., and then poured onto 200 parts of ice. The gum which is precipitated is allowed to settle and the supernatant liquor is decanted. The gum is stirred with 35 parts of ether and methanol is gradually added until the gum crystallises. The crystalline product is filtered off, washed with ether and dried. The 5-hydroxy-6-nitrotrimellitic acid trimethyl ester so formed is a white solid melting at 140° C.

10 parts of this nitro ester are stirred with 24 parts of octadecyl iodide and 4.8 parts of freshly prepared dry silver oxide at 100° C. for 30 minutes. The precipitate of silver iodide is filtered off and washed with ether and the filtrate and washings are heated to evaporate off the ether. 40 parts of methanol are added to the residue left after removal of the ether and 30% aqueous sodium hydroxide is then gradually added until the mixture remains alkaline (pH greater than 10) after boiling for 5 minutes. 100 parts of water are then added and the

alkaline solution so obtained is extracted with 100 parts of ether, the aqueous layer is separated and again extracted with 100 parts of ether. The aqueous layer is separated and carefully neutralised by the addition of dilute hydrochloric acid. The buff coloured precipitate so formed is filtered off, washed with 10% brine and dried. A mixture of 5-octadecyloxy-6-nitro-trimellitic acid and its sodium salt is obtained as a light brown hard wax, of indefinite melting point.

- 10 10 parts of this wax, 50 parts of 35% hydrochloric acid, 20 parts of water and 10 parts of stannous chloride are boiled together under a reflux condenser for 30 minutes. The suspended oil initially present is replaced by a pale straw coloured flocculent precipitate. The suspension is cooled and filtered and the residue on the filter is washed with 15% hydrochloric acid, and then with water. The product is dried at room temperature and ground, to form a buff coloured solid. The product which appears to be the monosodium salt is used without further purification.
- 15 20 What I claim is:

1. Process for the production of colour photographic images which comprises developing an exposed gelatino-silver halide emulsion layer with a colour photographic developer containing a primary aromatic amine developing agent in the presence of a colour coupler of the formula:



35 wherein Z represents the atoms required to complete a nucleus selected from the class consisting of benzene and quinoline nuclei and R represents a member of the class consisting of hydrogen and an acyl group.

- 40 2. Process according to claim 1 wherein the colour coupler is present in the developing solution.
3. Process according to claim 1 wherein the colour coupler is present in the gelatino-silver halide emulsion layer.
- 45 4. A light sensitive gelatino-silver halide emulsion layer containing a colour coupler of the formula:



55 55 wherein Z represents the atoms required to complete a nucleus selected from the class consisting of benzene and quinoline nuclei and R represents a member of the class consisting of hydrogen and an acyl group.

- 60 5. A light sensitive gelatino-silver halide emulsion layer containing a colour coupler as defined in claim 4 which contains an alkyl chain of at least 5 carbon atoms and a solubilizing group selected from the class consisting of sulphonate and carboxylic acid groups.

- 65 6. A light sensitive, silver halide emulsion layer containing the octadecyl ester of 1-acetyl-4-carboxy- $\beta:\gamma$ -benzisoxazolone.

- 70 7. A light sensitive, silver halide emulsion layer containing 1-acetyl- $\beta:\gamma$ -benzisoxazolone-4-carboxyoctadecylamide.

8. The process of claim 1 wherein said color coupler is the octadecyl ester of 1-acetyl-4-carboxy- $\beta:\gamma$ -benzisoxazolone.

9. The process of claim 1 wherein said color coupler is 1-acetyl- $\beta:\gamma$ -benzisoxazolone-4-carboxyoctadecylamide.

- 75 10. A light sensitive, silver halide emulsion layer con-

taining  $\beta:\gamma$ -benzisoxazolone-4-carboxy-(2'-N-methyl-N-octadecylamino-5'-sulpho-benz)-amide.

11. A light sensitive, silver halide emulsion layer containing 4:6-dicarboxy-7-octadecyloxy benzisoxazolone.

12. The process of claim 1 wherein said color coupler is  $\beta:\gamma$ -benzisoxazolone-4-carboxy-(2'-N-methyl-N-octadecylamino-5'-sulpho-benz)-amide.

13. The process of claim 1 wherein said color coupler is 4:6-dicarboxy-7-octadecyloxy benzisoxazolone.

14. The process of claim 1 wherein said color coupler is a hydroxyquinoline-isoxazolone.

References Cited in the file of this patent

UNITED STATES PATENTS

2,124,612 Eggert et al. July 26, 1938  
2,331,326 Kendall et al. Oct. 12, 1943